

March 8, 1938.

C. M. STEELE

2,110,455

MINE CAR WHEEL AND METHOD OF MAKING THE SAME

Filed Aug. 13, 1936

2 Sheets-Sheet 1



*Fig. 2.*



*Fig. 3.*



*Fig. 4.*



INVENTOR.

Charles M. Steele  
by  
Stebbins, Blenko  
his attorneys & Parmelee.

March 8, 1938.

C. M. STEELE

2,110,455

MINE CAR WHEEL AND METHOD OF MAKING THE SAME

Filed Aug. 13, 1936

2 Sheets-Sheet 2

Fig. 5.



Fig. 6.



Fig. 7.



Fig. 8.



INVENTOR

Charles M. Steele

by  
Stebbins, Blenko & Parmelee  
his attorneys

## UNITED STATES PATENT OFFICE

2,110,455

## MINE CAR WHEEL AND METHOD OF MAKING THE SAME

Charles M. Steele, North Irwin, Pa., assignor to  
Irwin Foundry & Mine Car Company, Irwin,  
Pa., a corporation of Pennsylvania

Application August 13, 1936, Serial No. 95,802

2 Claims. (Cl. 295—28)

This invention relates to an improvement in cast-iron car wheels, and more particularly for such wheels used on mine cars.

An object of the invention is to improve the 5 wearing qualities of the wheel. A further object is to improve the wearing qualities of the wheel while at the same time increasing its strength and resistance to shock.

In the accompanying drawings which illus- 10 trate my invention:

Figure 1 is a central vertical section through a mold flask for casting an improved wheel embodying my invention;

Figure 2 is a bottom perspective view of the 15 annular chill forming a part of the flask shown in Figure 1;

Figure 3 is a bottom perspective view of a baked core with segmental chills embedded in its periphery;

20 Figure 4 is a top plan view of the baked core shown in Figure 3, partially broken away to show a segmental chill embedded therein;

Figure 5 is a view in side elevation of the cast mine car wheel.

25 Figure 6 is a sectional view taken on the line VI—VI of Figure 5;

Figure 7 is a fragmentary sectional view illustrating the relation of the inner and outer chills to the tread of the wheel, this view being taken 30 on the line VII—VII of Figure 6 with the chills added;

Figure 8 is a cross section through the tread and the chills taken on the line VIII—VIII of Figure 7.

35 The present invention has grown out of the increasing demands placed upon mine car wheels. Mine cars are carrying heavier loads while at the same time the diameter of the wheels has remained the same or has even been decreased. 40 Consequently, the wearing away of the treads of the wheels has decreased the life of the wheels to such an extent as to become a problem.

Cast-iron wheels have the advantage that the 45 tread may be chill-cast. It is the chilled portion of the rim of the wheel which resists wear, and therefore, the thickness of the chilled tread determines the length of life of the wheel. In accordance with the present invention, the depth of chill of the tread is increased by using both 50 an inner chill and an outer chill for the tread when casting the wheel.

In setting up the mold flask shown in Figure 1 for casting the car wheel, I prefer to prepare the cope 10, the cores 11 and 12 and the drag 13 separately. The cope is provided with the usual

ribs 15 for maintaining the sand therein when the cope is lifted to its position on the other parts of the flask. The patterns for forming the green sand in the cope and drag are not shown, since this sand will be compacted in the cope and in the drag in the usual manner so as to present the upper and lower mold cavity surfaces as indicated in Figure 1. The drag may rest upon any suitable support such as the plate 16 shown in Figure 1.

10 The core 12 presents features of novelty in that segmental chills 18 are embedded in the sand, after which the core is baked with these chills embedded therein. A two-part mold is preferably employed for forming this core 12, as 15 will be understood by those skilled in this art.

It will be noted from Figure 1 that the flask is arranged for casting the wheel 20 with the flange 21 downwardly. Part of the flange is formed in the sand of the drag 13 and the remainder of the flange 21 is formed by an annular recess 23 along the lower inner portion of the annular chill 24.

The flask is assembled with the annular chill 24 intermediate the cope 10 and the drag 13, the 25 core 11 extending vertically through the center of the mold cavity, and the core 12 arranged coaxially with the annular chill 24. A gate through the central portion of the top of the cope is provided for pouring the molten metal 30 into the mold cavity. The molten metal fills the mold cavity and the excess metal forms the customary sprues. The impurities which go to make up the segregate tend to rise, so that the flange 21 is formed of purer metal than is the case 35 when the flange is cast uppermost.

The resulting wheel 20 is illustrated by Figures 5 to 8 of the drawings. The hub portion 26 is merely illustrative, for its form can be varied to provide the type of bearing desired. The rim 40 portion 27 includes the chilled tread 28, the flange 21, and a shoulder 29 which forms, at the other side of the tread from the flange 21, a continuation of the tread.

Between the central hub portion 26 and the 45 rim portion 27 extends a connecting portion 31, which is integral with the hub portion and the rim portion. This connecting portion does not follow established practice, because I leave open spaces or recesses beneath the tread 28 to accommodate the segmental chills 18 during casting. In accordance with my novel arrangement of this connecting portion, I support the hub portion 26 from the rim portion 27 in part by a web 32 and in part by spokes 33.

10

5

15

20

25

30

35

40

45

50

55

In the embodiment shown, the web 32 takes the form of a disc cast integral with the hub portion 26 and the flange 21. It is desirable to extend openings or perforations 34 through this disc, since the projections 35 on the core 12 which form these perforations 34 afford convenient means for resting the baked core 12 on the top surface of the green sand in the drag 13. The spokes 33 are cast integral with the hub portion 26 at 37 and extend to the rim portion 27, being integrally connected with the shoulder 29. These spokes include a portion 33, which extends across to the disc or web 32. This arrangement accords with my purpose of having the spokes recessed beneath the wheel tread.

Figures 7 and 8 illustrate the effect of the inner and outer chills on the grain structure of the tread. The outer chill hardens the cast metal both on the wearing surface of the tread and on the wearing surface of the flange. Due to the use of the inner chills 18, the body of hardened metal extends substantially completely through the tread so that the wear-resisting metal continues to be exposed by the wearing away of the surface of the tread until the rim portion 27 is too much worn away for further use of the wheel.

The unhardened metal in the rim portion 27 has an important function in the wheel. The hardened metal is brittle, and while it is highly wear-resistant it does not have the strength of the unhardened metal. The latter extends outwardly along the outer side of the flange 21 and into the shoulder 29 to reinforce the hardened metal in the tread 28.

A wheel embodying my invention has, therefore, the advantage of resistance to wear to the

very end of the life of the wheel without sacrificing toughness and ability to withstand shocks.

The form of wheel shown is to a large extent illustrative merely of the invention. As has been above mentioned, the design of the hub portion can be varied so that the desired type of bearing may be employed. It is not necessary that the inner chill be removed from the wheel after casting, since this chill could be left as a part of the finished wheel. In such a case, a solid ring 10 would be embedded in the core 12 and the wheel cast about this solid ring. It will be understood, therefore, that while I have illustrated and described the embodiment of my invention which I at present prefer, the invention may be otherwise embodied and practiced within the scope of the following claims.

I claim:

1. A car wheel having a hub portion, a rim portion including a flange and the wheel tread, 20 and a connecting portion extending between the hub portion and the rim portion and integral therewith wherein said connecting portion and the outer part at least of the flange are substantially without chill as cast and said tread is chilled 25 both from within and from without.
2. A car wheel having a hub portion, a rim portion including the wheel tread, a flange on one side of the tread and a shoulder forming a continuation at the other side of the tread, and 30 a connecting portion extending between the hub portion and the rim portion wherein said connecting portion, said shoulder and the outer part at least of the flange are substantially without chill as cast and said tread is chilled both 35 from within and from without.

CHARLES M. STEELE.